

Patented Dec. 27, 1932

1,892,051

# UNITED STATES PATENT OFFICE

DANIEL GRAY, OF ONEIDA, AND BURDETTE K. NORTHROP, OF HAMILTON, NEW YORK,  
ASSIGNORS TO ONEIDA COMMUNITY, LIMITED, OF ONEIDA, NEW YORK, A CORPORATION OF NEW YORK

## ELECTROPLATED CHROMIUM ARTICLE

No Drawing.

Application filed February 14, 1929. Serial No. 340,012.

This invention relates to improvements in the art of electroplating metals and metallic objects and articles.

The invention is intended to produce an improved process for electroplating or coating a metal having a passive surface, or surface film of impurities. The surface film impedes the adherence of electrodeposited metal to the base metal and prevents intimate union of the metallic coating with the raw metal beneath the film.

Surface films come on metals due to oxidation, sulphurization, or other forms of tarnishing or corrosion. Practically all metals, to some extent, take on such surface films, but the rapidity of formation varies with the different metals. Some metals produce surface films relatively slowly, while other metals form such films rapidly,—almost immediately, in some cases. In a metal of the former class, the coating can be applied directly to the surface. In the present practise, the metal is first thoroughly cleaned and all foreign matter removed from the surface.

The cleaned metal is then dipped in the plating bath and the plating or coating applied. The surface of the metal remains clean long enough to enable the coating to be applied and the coating metal to adhere to the raw, base metal. In a metal of the latter class, the surface film forms so quickly that it is impossible to apply the coating before formation of the film. The ordinary process for electroplating does not, therefore, work well with a metal of this class, as the coating does not adhere firmly due to the presence of the film.

Our present invention produces a process by which a metallic coating is made to adhere to the surface of a metal having a passive surface or a surface film. In its fundamental aspect, the invention resides in the use of an acid plating bath, in contradistinction to alkaline baths such as have been hitherto universally employed. In addition

to supplying the ions for the metallic coating, the acid bath eats into the surface of the base metal sufficiently to remove the surface film and expose the raw metal beneath, to which the metallic coating adheres firmly. In other words, the surface film is removed by the acid bath simultaneously with the deposition of the metallic coating.

In the preferred embodiment of the invention, the plating bath is strongly acid and contains a small amount of metal in solution for decomposition in the process and for supplying the coating. The metal to be plated or coated is dipped in the bath having the characteristics mentioned for a short time so that a thin layer of the coated metal is formed thereon and the acid does not act long enough to impair the metal. After this thin coating has been applied, the metal is quickly rinsed and washed so as to remove all traces of acid. The coating metal selected is such that it can, in turn, be plated in the usual manner, by the use of alkaline baths, and further coatings may be built up on it, until the finishing layer is obtained.

The invention will now be further illustrated with chromium taken by way of example to which the improved process is applied. It is to be understood, however, that the invention is also applicable in the electroplating of other metals, which present passive surfaces or surface films preventing firm adherence of coatings to the base metals.

Attempts to plate chromium with silver, copper or other metals, have hitherto met with failure because the passive surface or surface film of the chromium made it difficult to cause the electrodeposited coating to adhere thereto. Our present invention overcomes this difficulty and the plating is caused to adhere by "striking" the chromium with a metal, preferably copper, in an acid solution, preferably strong hydrochloric acid (C. P. HCl) containing a very small amount of copper chloride. In this way, a very thin

layer of copper is firmly affixed to the chromium surface and on this layer further metallic layers can be built up in the customary manner without difficulty.

5 The copper strike or bath may be made up as follows:— Twenty cubic centimeters (20 c. c.) of a stock copper chloride solution, (one gram of copper metal to the twenty cubic centimeters) are added to a four (4) 10 liter beaker nearly full of hydrochloric acid, C. P. HCl. Commercial hydrochloric acid will not work so well. No water is added. The solution thus obtained is employed as the copper "strike" bath. The solution provides a strong acid plating bath with a small amount of metallic or copper ions for decomposition therefrom and deposition on the chromium as a coating.

15 Preferably, two sheet copper anodes (each 20 1 1/2" x 9") are used with the above copper strike.

20 The current is preferably connected before hand and the chromium is allowed to remain in the bath or "strike" for about three seconds with full current flowing at around 9 or 25 10 volts. A thin bright deposit of copper is then obtained on the chromium.

25 The chromium is now removed, is washed and rinsed quickly and is promptly passed 30 into a warm copper cyanide bath. It is preferably allowed to remain in the cyanide bath for about 4 seconds with full current flowing at around 9 or 10 volts. The cyanide bath gives a thicker copper coating to the surface 35 and in this way the chromium is copper plated. The cyanide bath may be usual or stock composition.

40 If silver plating is desired, the same can be built up on the copper layers. The silver is also preferably applied in coatings or layers, the first of which is rather thin and the second thick. The first is preferably obtained by a silver cyanide "strike", with full current flowing at around 9 or 10 volts and for about 45 4 seconds. The silver "strike" may be a solution which contains .18 to .23 ounces of silver per gallon and 9 to 10 ounces of potassium cyanide per gallon. This composition is to be taken merely by way of example. The silver 50 "strike" provides a thin silver deposit on top of the copper and to this thin silver layer the full silver deposit can be applied and will adhere firmly.

55 The use of the acid "strike" or bath makes it possible to plate the chromium. The acid eliminates the passive surface condition or surface film of the chromium, and the solution provides the copper or other metallic ions which come into direct contact with the raw 60 chromium metal beneath the surface, adhere firmly thereto and provide the coating. The solution selected by way of example is a copper acid solution, for copper is a metal in common use in electroplating. Other metals 65 might be used as well. In general, the metal

selected to provide the initial thin coating should be such that other metallic coatings can be made to adhere thereto by the usual alkaline baths so that a coating sufficiently thick may be built up.

70 What is claimed is:

An electroplated product comprising a base of chromium, a coating of copper firmly adhering to the chromium, and a coating of silver firmly adhering to the copper coating.

75 In testimony whereof, we have hereunto set our hands.

DANIEL GRAY.  
BURDETTE K. NORTHROP.

80

85

90

95

100

105

110

115

120

125

130